

## UNITED STATES PATENT OFFICE

2,330,239

## LUBRICANT

Carl F. Prutton, Cleveland Heights, Ohio, assignor to The Lubri-Zol Corporation, Wickliffe, Ohio, a corporation of Ohio

No Drawing. Application November 25, 1940,  
Serial No. 367,031

21 Claims. (Cl. 252—53)

This invention relates, as indicated, to lubricating compositions and more particularly to lubricating compositions which are predominantly hydrocarbon oil, the properties of which affecting its use for particular purposes are improved by the addition of materials which are particularly effective in rendering the lubricants suitable for use under conditions of extreme stress as imposed by high temperatures, high loads, etc.

In my co-pending applications, Ser. No. 737,070, filed July 26, 1934, 216,153, filed June 27, 1938 and 245,226, filed December 12, 1938, I have disclosed a broad class of lubricating compositions of general utility, particularly in the field of use where extreme pressures are encountered.

My present invention relates to the discovery that a certain class of such materials is particularly suitable for use in lubricants subjected to conditions of extreme stress such as those involved in the lubrication of heavily loaded gears, and in the lubrication of internal combustion engines operating under severe service conditions; for example, those encountered by internal combustion engines particularly of the aviation and Diesel types.

It is the principal object of my invention, therefore, to provide a lubricating composition which is especially suited for the purposes described.

Other objects of my invention will appear as the description proceeds.

To the accomplishment of the foregoing and related ends, said invention, then, consists of the means hereinafter fully described and particularly pointed out in the claims; the following description setting forth in detail certain approved combination of ingredients embodying my invention, such disclosed combinations of ingredients embodying my invention, such disclosed means constituting, however, but one of various forms in which the principle of the invention may be used.

Broadly stated, this invention comprises the provision of a lubricating composition for the purposes specified, characterized by the fact that the same contains a lubricating oil, preferably of the hydrocarbon type, as a major constituent with the properties of such composition affecting its use as a lubricant, especially under the conditions specified, by the incorporation therein of a minor amount, based on the amount of lubricating oil present, of a stable, oil-soluble salt of an aromatic acid.

More especially, my invention comprises the discovery that salts of aromatic acids, of the type which contain a substituent selected from the class consisting of aliphatic and cyclo-aliphatic radicles, are particularly suited for use.

*The oil base*

The oil base of my lubricating compositions is a lubricating oil of the type best suited for the particular use for which the ultimate composition is designed. When the lubricating compositions of my invention are designed for the lubrication of automobiles, the oil base will of course preferably consist of a refined mineral lubricating oil of lubricating viscosity for the particular point of application. In other words, a conventional gear oil may be used for the lubrication of the gears and generally a lighter, more highly refined, oil will be used in the crank case.

15 This invention is applicable to lubricating compositions in which the base may consist either entirely or in part of synthetic oils, hydrogenated oils, and volatilized oils.

16 The oil base may also desirably contain other well known constituents such as those which improve the oiliness, film strength, pour point, cold test, corrosiveness, and oxidation properties, etc., of the oil. In general, compositions of my invention may be employed with any commercially 20 available addition agents for the above defined purposes since they are generally compatible with the same in the amounts usually used.

*The addition agents*

25 As above indicated, the addition agents may be generally defined as salts of aromatic acids. The term salts as used herein is intended to include the salts formed by organic bases with aromatic acids as well as the salts formed by inorganic bases with aromatic acids. The inorganic base salts such as the metallic salts of aromatic acids will generally be found to give best results, and of these, those salts in which the metal is present in polyvalent and especially in divalent form, 30 will usually be preferred.

The halogen bearing salts of aromatic acids generally are a broad class of addition agents which have been found to be notably effective.

35 For certain uses, the salts of aromatic acids of the type which contain a substituent selected from the class consisting of aliphatic radicles and cyclo-aliphatic radicles have been found very useful. This latter class of salts may optionally 40 also contain a halogen such as chlorine.

45 Due to the nature of the addition agents contemplated for use, they may be conveniently identified by first having reference to the various aromatic acids from which the salts may be prepared and by then giving a list of the various 50 radicles or bases which may be combined with such acids in producing the salts.

TABLE I.—AROMATIC ACIDS

## A. Aromatic acids with carboxyl group attached to ring

|                                                                            |    |                                                       |
|----------------------------------------------------------------------------|----|-------------------------------------------------------|
| Benzoic acid                                                               | 5  | (2) With substituent attached to nitrogen atom, e. g. |
| Benzoic acid derivatives:                                                  |    | N-alkylated anthranilic acids                         |
| Hydroxybenzoic acids                                                       |    | N-methyl anthranilic acids                            |
| p-Hydroxybenzoic acid                                                      |    | N-dimethyl anthranilic acids                          |
| Salicylic acid                                                             |    | N-amyl anthranilic acids                              |
| Polyhydroxybenzoic acids                                                   |    | N-lauryl anthranilic acids                            |
| Protocatechuic acid                                                        |    | N-dilauryl anthranilic acids                          |
| Pyrocatechuic acid                                                         |    | N-ceryl anthranilic acids                             |
| Resorcylic acids                                                           |    | N-acetyl anthranilic acids                            |
| Gallic acid                                                                |    | N-stearoyl anthranilic acids                          |
| Amino-benzoic acids                                                        | 10 | N-naphthyl anthranilic acids                          |
| p-Aminobenzoic acid                                                        |    | N-phenyl anthranilic acid                             |
| Anthranilic acid                                                           |    | N-diphenyl anthranilic acid                           |
| Azobenzene acids                                                           |    | N-benzoyl anthranilic acid                            |
| Thiobenzoic acids                                                          | 15 | N-naphthyl anthranilic acid                           |
| Monothiobenzoic acid (Sulphydryl benzoic acids)                            |    | Benzene polycarboxylic acids                          |
| Dithiobenzoic acid                                                         |    | Phthalic acid                                         |
| Mercapto benzoic acids (Thio-salicylic acid (o-mercapto-benzoic acid))     |    | Isophthalic acid                                      |
| p-Mercapto-benzoic acid                                                    |    | Terephthalic acid                                     |
| Alkylated benzoic acids                                                    | 20 | Benzene tricarboxylic acids                           |
| Methyl benzoic acids                                                       |    | Benzene tetracarboxylic acids                         |
| Toluic acids                                                               |    | Diphenyl carboxylic acids                             |
| Xylic acids                                                                |    | Phenyl benzoic acids                                  |
| Trimethyl benzoic acids                                                    |    | Diphenic acid                                         |
| Ethyl benzoic acids                                                        |    | Diphenylmethane carboxylic acids                      |
| Lauryl benzoic acids                                                       |    | o-Benzyl benzoic acid                                 |
| Cetyl benzoic acids                                                        |    | Benzyl phthalic acids                                 |
| Carnaubyl benzoic acids                                                    | 25 | Benzophenone carboxylic acids                         |
| Ceryl benzoic acids                                                        |    | o-Benzoyl benzoic acid                                |
| Montanyl benzoic acids                                                     |    | Benzoyl phthalic acids                                |
| Myricyl benzoic acids                                                      |    | Naphthalene carboxylic acids                          |
| Cyclo-aliphatic substituted benzoic acids                                  | 30 | Alpha-naphtholic acid                                 |
| Cyclohexyl-benzoic acid                                                    |    | Beta-naphtholic acid                                  |
| Methyl-cyclohexyl benzoic acids                                            |    | Naphthalene polycarboxylic acids                      |
| Amyl-cyclohexyl benzoic acids                                              |    | Naphthalic acid                                       |
| Naphthylbenzoic acids                                                      |    | Anthracene carboxylic acids                           |
| Naphthoyl benzoic acids                                                    |    | Anthraquinone carboxylic acids                        |
| Ether-substituted benzoic acids                                            | 35 | Phenanthrene carboxylic acids                         |
| Methoxy-benzoic acids                                                      |    | Heterocyclic acids                                    |
| Ethoxy-benzoic acids                                                       |    | Furan carboxylic acids                                |
| Lauroxy-benzoic acids                                                      |    | Furoic acid (pyromuic acid)                           |
| Phenoxy-benzoic acids                                                      |    | Pyrrole carboxylic acids                              |
| Veratric acid                                                              |    | Pyrrole alpha-carboxylic acid                         |
| Piperonylic acid                                                           |    | Thiophene carboxylic acids                            |
| Keto-substituted benzoic acids                                             | 40 | Thiophene alpha-carboxylic acid                       |
| Acetyl benzoic acids                                                       |    | Thiophene beta-carboxylic acid                        |
| Lauroyl benzoic acids                                                      |    | Pyridine carboxylic acids                             |
| Stearoyl benzoic acids                                                     |    | Picolinic acid                                        |
| Naphthoyl benzoic acids                                                    |    | Nicotinic acid                                        |
| Benzoyl benzoic acids                                                      |    | Pyridine polycarboxylic acids                         |
| Ester-substituted benzoic acids                                            | 45 | Pyridine dicarboxylic acids                           |
| Mono-esters of phthalic acid, isophthalic acid and terephthalic acid       |    | Quinolinic acid                                       |
| (ROOC—C <sub>6</sub> H <sub>4</sub> —COOH)                                 |    | Lutidinic acid                                        |
| Mono-methyl phthalate                                                      |    | Dinicotinic acid                                      |
| Mono-amyl phthalate                                                        |    | Dipicolinic acid                                      |
| Mono-lauryl phthalate                                                      |    | Cinchonemic acid                                      |
| Mono-benzyl phthalate                                                      |    | Isocinchonemic acid                                   |
| Mono-cyclohexyl phthalate                                                  |    | Pyridine 2,3,6, tricarboxylic acid                    |
| Amide-substituted benzoic acids                                            | 50 | Quinoline carboxylic acids                            |
| Mono-amides of phthalic acid, isophthalic acid, and terephthalic acid      |    | Quinaldinic acid                                      |
| R—NCO—C <sub>6</sub> H <sub>4</sub> —COOH                                  |    | Cinchoninic acid                                      |
| R—NCO—C <sub>6</sub> H <sub>4</sub> —COOH and                              |    | Quinilic acid                                         |
| R—NCO—C <sub>6</sub> H <sub>4</sub> —COOH                                  |    | Acridinic acid                                        |
| N-Methyl phthalic acid mono-amide                                          | 55 |                                                       |
| N-Amyl phthalic acid mono-amide                                            |    |                                                       |
| N-Lauryl phthalic acid mono-amide                                          |    |                                                       |
| N-Cyclohexyl phthalic acid mono-amide                                      |    |                                                       |
| N-Methyl cyclohexyl acid mono-amide                                        |    |                                                       |
| Thio-amide substituted benzoic acids                                       | 60 |                                                       |
| Mono thio-amides of phthalic acid, isophthalic acid, and terephthalic acid |    |                                                       |
| R—NH <sub>2</sub> CS—C <sub>6</sub> H <sub>4</sub> —COOH and               |    |                                                       |
| R—NH <sub>2</sub> CS—C <sub>6</sub> H <sub>4</sub> —COOH                   |    |                                                       |
| R—NCS—C <sub>6</sub> H <sub>4</sub> —COOH                                  |    |                                                       |
| R—NCS—C <sub>6</sub> H <sub>4</sub> —COOH                                  |    |                                                       |
| e. g. where R and R' are:                                                  |    |                                                       |
| Methyl, amyl, lauryl, cyclohexyl, methyl cyclohexyl, etc.                  |    |                                                       |
| Salicylic acid derivatives:                                                | 65 |                                                       |
| Alkylated salicylic acids                                                  |    |                                                       |
| Ethyl salicylic acids                                                      |    |                                                       |
| Lauryl salicylic acids                                                     |    |                                                       |
| Cyclohexyl salicylic acids                                                 |    |                                                       |
| Naphthyl salicylic acids                                                   |    |                                                       |
| Stearoyl salicylic acids                                                   |    |                                                       |
| Anthranilic acid derivatives:                                              | 70 |                                                       |
| (1) With substituent in ring e. g.                                         |    |                                                       |
| Alkylated anthranilic acids                                                |    |                                                       |
| Propyl anthranilic acids                                                   |    |                                                       |
| Amyl anthranilic acids                                                     |    |                                                       |
| Lauryl anthranilic acids                                                   |    |                                                       |
| Phenyl anthranilic acids                                                   |    |                                                       |
| Benzoyl anthranilic acids                                                  |    |                                                       |
| Stearoyl anthranilic acids                                                 |    |                                                       |
| Hydroxy-phenyl anthranilic acids                                           |    |                                                       |

**B. Aromatic acids containing fatty-acid radicles having a plurality of carbon atoms—Cont.**

Aromatic myristic acids  
Phenyl myristic acid  
Naphthyl myristic acid  
Aromatic palmitic acids  
Phenyl palmitic acid  
Naphthyl palmitic acid  
Xenyl palmitic acid  
Tolyl palmitic acid  
Xylyl palmitic acid  
o-Hydroxyphenyl palmitic acid  
o-Benzoylphenyl palmitic acid  
Stearoyl-phenyl palmitic acid  
Aromatic stearic acids  
Phenyl stearic acid  
Diphenyl stearic acid  
Triphenyl stearic acid  
Xenyl stearic acid  
Naphthyl stearic acid  
o-Cyclohexyl-phenyl stearic acid  
Tolyl stearic acid  
Xylyl stearic acid  
Ethyl-phenyl stearic acid  
Lauryl-phenyl stearic acid  
Benzyl stearic acid  
Benzoyl stearic acid  
o-Hydroxy-phenyl stearic acid  
p-Hydroxy-phenyl stearic acid  
Hydroxy-xenyl stearic acids  
Dihydroxy-phenyl stearic acids  
Amino-phenyl stearic acids  
N-lauryl-amino-phenyl stearic acids  
N-cyclohexyl-amino-phenyl stearic acids  
N-dilauryl-amino-phenyl stearic acids  
Salicyl stearic acids  
Benzoyl-phenyl stearic acids  
Stearoyl-phenyl stearic acids  
Phenoxy-phenyl stearic acids  
Methoxy-phenyl stearic acids  
Lauroxy-phenyl stearic acids  
Furyl stearic acid  
Pyridyl stearic acid  
Phenyl hydroxystearic acid  
Phenyl glyoxylic acid  
Benzoyl glycolic acid  
Hippuric acid  
Phenyl glycine  
Phenyl glycine o-carboxylic acid  
Phenyl alanine  
Benzilic acid  
Phthalonic acid  
N-phenyl succinamic acid  
N-diphenyl succinamic acid  
Benzyl tartronic acid  
Aromatic unsaturated acids  
Acrylic acid  
Cinnamic acid  
Cumaric acid  
Phenyl angelic acid  
Phenyl cinnamic acid  
Phenyl crotonic acid  
Phenyl-amino crotonic acid  
Phenyl propiolic acid  
Benzoyl acrylic acid  
Phenyl oleic acids  
Phenyl ricinoleic acid  
Benzal lactic acid  
Benzal malonic acid  
Fural malonic acid  
Benzal propionic acid

**C. Aromatic cyclo-aliphatic acids**

Aromatic derivatives of naphthenic acids  
Phenyl naphthenic acids  
Hydroxy-phenyl naphthenic acids  
Benzyl naphthenic acids  
Benzoyl naphthenic acids  
Naphthyl naphthenic acids  
Xenyl naphthenic acids  
Aromatic derivatives of cyclopropane carboxylic acids  
Phenyl-ethylene acetic acid  
Phenyl-vinacetic acid  
Phenyl caronic acid  
Aromatic derivatives of cyclo-butane carboxylic acids  
Truxillie acids  
Truxinic acids  
Phenyl norpinic acid  
Phenyl pinic acid  
Aromatic derivatives of cyclopentane carboxylic acids  
Phenyl camphoric acid  
Phenyl camphenic acid  
Phenyl 2,3,4-trimethyl cyclopentane-3 carboxylic acid  
Aromatic derivatives of cyclohexane carboxylic acids  
Phenyl hexa-hydrobenzoic acids  
Hydroxy-phenyl hexahydrobenzoic acids  
Benzyl hexahydrobenzoic acids  
Benzoyl hexahydrobenzoic acids  
Naphthyl hexahydrobenzoic acids  
Phenyl hexahydrophthalic acids  
Benzoyl hexahydrophthalic acids  
Hydroxy-phenyl hexahydrophthalic acids  
Phenyl quinic acid

**D. Aromatic acids other than carboxylic**

Hydroxyl-containing derivatives of benzene  
Pyrogallic acid  
Pyrogallic acid derivatives  
5 Alkylated pyrogallic acid  
Lauryl pyrogallic acid  
Esters of gallic acid  
Methyl gallate  
Amyl gallate  
Lauryl gallate  
Phenyl gallate  
Benzyl gallate  
Cyclohexyl gallate  
10 Methyl-cyclohexyl-gallate  
Amides of gallic acid  
Gallic acid amide  
Gallic acid anilide  
N-lauryl gallic acid amide  
Hydroxyl-containing derivatives of triphenyl methane  
Pararosolic acid  
15 Rosolic acid  
Mercapto-rosolic acid  
Thio-rosolic acids  
Any of the acids listed above under A, B, C, and D in which one or more oxygen atoms have been replaced with sulphur. Any of the foregoing which have been halogenated or in which one or more hydrogen atoms have been replaced with a halogen.  
20 In the preparation of those salts of aromatic acids of the type in which the aromatic acid is of the class which contains a substituent selected from the class consisting of aliphatic radicles and cyclo-aliphatic radicles, such acids 25 may be conveniently prepared either by:  
(1) Condensing an aromatic compound with  
(a) An aliphatic unsaturated acid, or  
(b) A halogenated aliphatic acid, or  
(c) A cyclo-aliphatic unsaturated acid, or  
(d) A halogenated cyclo-aliphatic acid; or by  
30 (2) Condensing an aromatic acid with  
(a) An unsaturated aliphatic compound, or  
(b) A halogenated aliphatic compound, or  
(c) An unsaturated cyclo-aliphatic compound, or  
(d) A halogenated cyclo-aliphatic compound.

Aromatic compounds which may be used in 35 any of the condensation reactions identified under (1) above in the preparation of aromatic acids from which appropriate salts may be prepared are as follows:

**TABLE II.—AROMATIC COMPOUNDS**

40 I. Hydrocarbons  
(A) Benzene and its homologs such as toluene, xylene, cymene, ethyl-benzene, mesitylene.  
(B) Polyprenyls such as diphenyl, diphenyl benzene, and homologs of them such as o-phenyl toluene, poly-ethyl diphenyls, propyl diphenyl.  
45 (C) Condensed ring hydrocarbons  
(1) Naphthalene and its homologs, such as the methyl naphthalenes, ethyl naphthalenes, propyl naphthalenes.  
(2) Phenanthrene and anthracene and their homologs such as the mono- and di-methyl, and propyl and iso-propyl, substitution products, e. g. retene.  
50 (3) Chrysene and picene and their homologs.  
(D) Compounds resulting from substitution of aryl groups in compounds of classes (A), (B) and (C), e. g., di-benzyl, di-naphthyl, phenyl naphthalenes, the polyphenylmethanes, etc.  
(E) Bridged ring hydrocarbons such as certain of the terpenes and related compounds including pinene, camphene and limonene.  
55 II. Heterocyclic compounds of the aromatic or allied type such as: pyridine, quinoline, etc. and their derivatives.  
III. Substitution products (other than hydrocarbon homologs) of compounds of classes I and II, including:  
(A) Oxygen-bearing substitution products. (See Table No. II(a) below, for further classification.)  
60 (B) Halogen-bearing substitution products.  
(C) Other substitution products, such as those resulting from substitution of the following groups:  
Amino, and substituted amino groups Mercapto  
Imino Sulphide  
Azo Polysulphide  
65 Hydrazo Thiocyanate  
Hydrazine Isothiocyanate  
Nitrile Dithiocarboxylic acids (also ester and salt groups derived therefrom)  
Isonitrile

IV. Derivatives of the compounds included in classes I, II, and III resulting from addition reactions, such as hydrogenation, halogenation, etc. Examples of such compounds are the hydro-naphthalenes, phenyl cyclohexane, phenyl cyclohexanol, cyclohexyl phenol, naphthalene tetrachloride.

70 Attention is called to the fact that certain of the compounds may belong to more than one class; as, for example, the halogenated phenols which belong in class III(A) and III(B), or the



Table No. 2

|                                 |                                  |
|---------------------------------|----------------------------------|
| (1) Unsaturated alcohols, e. g. | (2) Unsaturated aldehydes, e. g. |
| Vinyl ethyl alcohol             | Acrolein                         |
| Allyl alcohol                   | Crotonaldehyde                   |
| Crotonyl alcohol                | Hexadienal                       |
| Oleyl alcohol                   | Octaenial                        |
| Propargyl alcohol               | Citral                           |
|                                 | Propargylic aldehyde             |

## (3) Unsaturated ketones, e. g.

|                     |
|---------------------|
| Allyl acetone       |
| Di-allyl ketone     |
| Mesityl oxide       |
| Phorone             |
| Vinyl lauryl ketone |

Acetylenic ketones (e. g.  $R-C\equiv C-CO-R'$ ), such as:

|                        |
|------------------------|
| Allylene methyl ketone |
| Allylene lauryl ketone |

## (3a) Ketenes

## Ketene

## Acetyl ketene

## (4) Unsaturated ethers, e. g.

|                       |
|-----------------------|
| Di-vinyl ether        |
| Di-allyl ether        |
| Allyl ethyl ether     |
| Vinyl ethyl ether     |
| Allyl iso-amyl ether  |
| Allyl lauryl ether    |
| Propargyl ethyl ether |

## (5) Unsaturated acids, e. g.

|                             |
|-----------------------------|
| Vinyl acetic acid           |
| Vinyl acrylic acid          |
| Vinyl glycolic acid         |
| Acrylic acid                |
| Crotonic acid               |
| Oleic acid                  |
| Linoleic acid               |
| Maleic acid                 |
| Hydroxymaleic acid          |
| Fumaric acid                |
| Glutaconic acid             |
| Linolenic acid              |
| Elaeostearic acid           |
| Propiolic acid              |
| Stearoic acid               |
| Acetylene dicarboxylic acid |

## (5') Unsaturated anhydrides

|                             |
|-----------------------------|
| Maleic anhydride            |
| Itaconic anhydride          |
| Citraconic anhydride        |
| Pyrocinchoninic anhydride   |
| Xeronic anhydride           |
| Glutaconic anhydride        |
| Methyl glutaconic anhydride |
| Dimethyl anhydride          |

## (6) Unsaturated esters, e. g.

(a) Esters of unsaturated acids (e. g. those listed under (5) above as well as unsaturated aromatic acids such as cinnamic and coumaric) with mono- and poly-hydric alcohols, or other hydroxy compounds (including phenols). Examples of such alcohols and hydroxy compounds are:

|                                                    |
|----------------------------------------------------|
| Methyl alcohol                                     |
| Ethyl alcohol                                      |
| Propyl alcohol                                     |
| Butyl alcohols                                     |
| Amyl alcohols                                      |
| Lauryl alcohols                                    |
| Cetyl alcohols                                     |
| Cyclohexanol                                       |
| Alkylated cyclohexanols, e. g. methyl cyclohexanol |
| Benzyl alcohol                                     |
| Furfuryl alcohol                                   |
| Tetrahydrofurfuryl alcohol                         |
| Ethylene glycol                                    |
| Propylene glycol                                   |
| Di-ethylene glycol                                 |
| Glycerol                                           |
| Erythritol                                         |
| Phenol                                             |
| Polyhydroxy-benzenes                               |
| Alkylated phenols                                  |
| Naphthols                                          |

Unsaturated alcohols (e. g. those listed under (1) above)

(b) Esters of unsaturated alcohols (e. g. those listed under (1) above) with organic acids, either aliphatic or aromatic, or with inorganic acids. Examples of such acids are:

Aliphatic acids, including:

|                           |
|---------------------------|
| Saturated acids, such as: |
| Acetic acid               |
| Propionic acids           |
| Butyric acids             |
| Lauric acids              |
| Palmitic acid             |
| Stearic acid              |
| Oxalic acid               |
| Citric acid               |
| Laetic acid               |
| Glycolic acid             |
| Malonic acid              |
| Tartaric acid             |

Unsaturated acids, such as those listed under (5) above.

Aromatic acids, including:

|                 |
|-----------------|
| Benzonic acid   |
| Phthalic acids  |
| Salicylic acid  |
| Anthrancic acid |
| Cinnamic acid   |

Cyclo-aliphatic acids, including:

|                       |
|-----------------------|
| Naphthenic acids      |
| Hexahydrobenzoic acid |

## Heterocyclic acids including:

## Furoic acid

## Pyrrol carboxylic acids

## Pyridine carboxylic acids

## Inorganic acids, including:

## Hydro-halogen acids

## Oxy-halogen acids

## Sulphurous acid

## Sulphuric acid

## Thiosulphuric acid

## Carbonic acid

## Thiocarbonic acids

## Hydrogen sulphide

## Phosphorous acid

## Thiophosphorous acids

## Phosphoric acid

## Thiophosphoric acids

## Cyanic acid

## Thiocyanic acid

## Hydrocyanic acid

## Boric acid

## 15 (7) Salts of unsaturated acids, including the

## Ammonium and substituted ammonium

## Sodium

## Calcium

## Barium

## Cobalt

## Aluminum

## Magnesium

## Zinc

## Lead

Salts of unsaturated acids generally, and more specifically of such acids as those listed under (5) above and of unsaturated aromatic acids.

In addition to the compounds listed above, commercial products comprising complex mixtures of unsaturated oxygen-bearing organic compounds may be used as the "unsaturated" reactant. Examples of such materials are the fatty oils of unsaturated character, e. g.

|                |                   |
|----------------|-------------------|
| 30 Castor oil  | Linseed oil       |
| Chinawood oil  | Menhaden fish oil |
| Corn oil       | Rape seed oil     |
| Cottonseed oil | Soya bean oil     |
| Coconut oil    | Sperm oil         |
| Lard oil       |                   |

Additional material, for use as the "unsaturated" reactant in the condensation, may be derived from any of the above fatty oils, e. g.

- Acids, extracted from the oils by direct hydrolysis, or by saponification and subsequent hydrolysis, or otherwise.
- Esters, produced by esterifying the acids of (1) in Table No. 2.
- Soaps, produced by saponifying the oils directly or by neutralizing the acids of (1) with alkalies, e. g. to form salts analogous to those listed under (7) in Table No. 2.

The unsaturated oxygen compounds are of particular importance and may, therefore, be classified in further detail according to the nature of the attachment of the oxygen atom to the molecule, viz:

Table No. 3

## 50 I'. Directly attached to one or more carbon atoms, as in the case of:

## (1') Ethers and analogous compounds

## (2') Compounds containing the



radicle, such as alcohols and other derivatives of carbinol (including phenols, cresols, naphthols, etc.)

## (3') Compounds containing the carbonyl



radicle, such as amides, aldehydes, ketones, organic acids, esters and salts of organic acids (including such salts of both inorganic and organic bases), thio-acids and esters and salts of thio-acids.

## (4') Compounds in which oxygen forms a part of a ring structure, e. g. compounds containing the furyl or hydro-furyl groups.

## (5') Compounds with an inorganic radicle where the oxygen is directly attached to a carbon atom, e. g.

## Arsenites

## Hypochlorites

## Phosphites

## Thiophosphates

## Thiophosphites

## S-Hydroxylamines

## Borates

## 65 II'. Indirectly attached through the means of some other atom, i. e., in the form of an inorganic radicle, e. g.

## Arsenate

## Chlorate

## Chlorite

## Cyanate

## a-Hydroxylamine

## Nitrate

## Nitrite

## Nitro

## Nitroso

## Oxime

## Perchlorate

## Phosphate

## Sulphite

## Sulphite

## Sulphonic acid

## Sulphone

## Sulphoxide

## Thiophosphate

## Thiophosphite

## Thio-sulphate

(Note.—This class includes salts of organic bases with inorganic oxy-acids.)

In the following table are listed a number of representative halogenated aliphatic compounds which may be used as one of the components of the condensation reaction identified under (2) (b) above.

TABLE VIII.—HALOGENATED ALIPHATIC COMPOUNDS

|                    |                      |
|--------------------|----------------------|
| Ethyl chloride     | Benzyl chloride      |
| Butyl chloride     | Ethylene dichloride  |
| Amyl chloride      | Carbon tetrachloride |
| Lauryl chloride    | Chlorparaffin wax    |
| Cetyl chloride     | Chlor naphtha        |
| Ceryl chloride     | Chlor decane         |
| Mellissyl chloride | Amyl dichloride      |

Chlorinated aliphatic paraffin derivatives as well as the chlorinated derivatives of the various materials and compounds listed in Table VII above.

In the following table are listed a number of specific examples of unsaturated cyclo-aliphatic compounds which may be employed as components of the condensation reaction identified under (2) (c) above.

TABLE IX.—UNSATURATED CYCLO-ALIPHATIC COMPOUNDS

Examples of such unsaturated cyclic compounds are:

Hydrocarbons:

Cyclobutene  
Methyl cyclobutene  
Methylene cyclobutane  
Cyclopentene  
Methyl cyclopentenes  
Laurolene  
Cyclopentadiene  
Fulvenes  
Di-cyclopentadiene  
Cyclohexene  
Methyl cyclohexenes  
Cyclohexadienes  
Methyl cyclohexadienes  
P-menthenes  
P-menthadienes  
Terphenenes  
Limonene  
Di-cyclohexadiene  
Dihydronaphthalene  
Dihydrodiphenyl  
Tetrahydrodiphenyl  
Pinenes  
Camphene

Oxygen-containing compounds

Alcohols  
Terpineol  
Isopulegol  
Dihydrocarveol  
Pinocarveol  
Aldehydes  
Ketones  
Pulegone  
Piperitone  
Carvone  
Eucarvone  
Ionone  
Pinocarvone  
Verbenone  
Carvenone  
Ethers  
Pinol  
Tetrahydro-anisole  
Tetrahydro-phenetole  
Acids  
Laurolenic acid  
Chaulmoogric acid  
Hydrocarpic acid  
Tetrahydrobenzole acid  
Tetrahydronthalic acid  
Tetrahydrotoluic acids  
Dihydroththalic acids  
Tetrahydro-xylic acids  
Methyl cyclohexylidene acetic acid  
Fural acrylic acid  
Fural malonic acid  
Benzal malonic acid  
Benzal propionic acid  
Benzal lactic acid  
Abietic acid

Commercial products comprising complex mixtures of unsaturated cyclic organic compounds may also be used, e. g.

Turpentine  
Pine oil

In the following table are listed a number of representative examples of halogenated cyclo-aliphatic compounds which may be employed as

one of the components of the condensation reaction identified under (2) (d) above.

TABLE X.—HALOGENATED CYCLO-ALIPHATIC COMPOUNDS

|    |                                          |
|----|------------------------------------------|
| 5  | Halogenated cyclo-aliphatic hydrocarbons |
|    | Chlorcyclobutane                         |
|    | Chlorcyclopentane                        |
|    | Chloretylecyclobutane                    |
|    | Chlorcyclohexane                         |
| 10 | Chloromethylcyclohexane                  |
|    | Dichlorcyclohexane                       |
|    | Chlorcycloparaffin                       |
|    | Dichlorcyclopentane                      |
|    | Halogenated cyclo-aliphatic alcohols     |
|    | Chlorcyclopentanol                       |
|    | Chlorcyclohexanol                        |
| 15 | Chloromethylcyclohexanol                 |
|    | Chlorquinitol                            |
|    | Chlormenthol                             |
|    | Chlor-terpins                            |
|    | Chlor-terpineols                         |
|    | Chlor-borneol                            |
|    | Halogenated cyclo-aliphatic ketones      |
| 20 | Chlorcyclobutanone                       |
|    | Chlorcyclobutyl methyl ketone            |
|    | Chlorcyclopentanone                      |
|    | Chlor-cyclohexanone                      |
|    | Chlormenthone                            |
|    | Chlor-camphor                            |
|    | Brom-camphor                             |
|    | Halogenated cyclo-aliphatic esters       |
| 25 | Chloromethyl-naphthenates                |
|    | Chlorcyclohexyl-acetate                  |
|    | Chlorcyclohexyl-stearate                 |
|    | Chloromethyl-hexahydrobenzoate           |
|    | Chlor di-methyl-hexahydrophthalate       |

The various aromatic acids, either those specifically identified in Table I above or those prepared by the various condensation reactions above identified, may, as previously indicated, be combined with either an organic radicle or base in the preparation of organic salts or with inorganic bases in the preparation of the inorganic salts.

In the following table will be found listed a number of organic radicles or bases which may thus be employed in the preparation of organic salts of aromatic acids.

40

TABLE XI.—ORGANIC RADICLES OR BASES

|    |                                   |
|----|-----------------------------------|
| 45 | Amino compounds such as:          |
|    | Monooethanolamine                 |
|    | Diethanolamine                    |
|    | Triethanolamine                   |
|    | Aniline                           |
|    | Benzylamine                       |
|    | Laurylamine                       |
|    | Diphenylamine                     |
|    | Triphenylamine                    |
| 50 | Diethylamine                      |
|    | Triethylamine                     |
|    | Putrescine                        |
|    | Nitrogen ring compounds, such as: |
|    | Pyrimidine                        |
|    | Pyrazine                          |
|    | Phenazine                         |

Oxygen-bearing ring compounds, such as:

55  $\gamma$ -Pyrone

Among the specific organic salts of aromatic acids which may thus be prepared for use, may be listed the following as illustrative examples.

60

TABLE XII.—ORGANIC SALTS

|    |                                     |
|----|-------------------------------------|
| 65 | Aniline phenyl stearate             |
|    | Benzylamine chlorophenylstearate    |
|    | Laurylamine naphthylstearate        |
|    | Diphenylamine chlorophenylstearate  |
|    | Diethylamine phenylmercaptostearate |
|    | Ethanolamine phenylpalmitate        |
|    | Triethanolamine piperidyl laurate   |
|    | Pyridine phenyl stearate            |
|    | Quinoline naphthyl palmitate        |
|    | Piperidine chlor naphthyl laurate   |
|    | Thiazole phenyl palmitate           |
|    | $\gamma$ -Pyrone phenyl stearate    |

70 In the following table are listed a number of inorganic radicles which may be combined with any of the aromatic acids given above in the production of inorganic salts of aromatic acids which may be used as addition agents in the lubricating compositions of my invention.

75

TABLE XIII.—INORGANIC RADICLES

|           |                            |
|-----------|----------------------------|
| Sodium    | Aluminum                   |
| Potassium | Chromium                   |
| Ammonium  | Stannous                   |
| Lithium   | Lead                       |
| Beryllium | Copper                     |
| Magnesium | Cadmium                    |
| Calcium   | Bismuth                    |
| Strontium | Silver                     |
| Barium    |                            |
| Cobalt    | Mercury                    |
| Zinc      |                            |
| Nickel    |                            |
| Manganese | Vanadyl (VO <sub>2</sub> ) |

In the following table are given a list of representative inorganic salts which may be produced by the combination of certain of the aromatic acids above identified with certain of the inorganic radicles of Table XIII above.

TABLE XIV.—INORGANIC SALTS

|                                        |
|----------------------------------------|
| Calcium diphenyl acetate               |
| Magnesium diphenyl acetate             |
| Nickel diphenyl acetate                |
| Cobalt diphenyl acetate                |
| Stannous diphenyl acetate              |
| Potassium phenyl stearate              |
| Ammonium phenyl stearate               |
| Lithium phenyl stearate                |
| Magnesium phenyl stearate              |
| Calcium phenyl stearate                |
| Strontium phenyl stearate              |
| Barium phenyl stearate                 |
| Cobalt phenyl stearate                 |
| Zinc phenyl stearate                   |
| Nickel phenyl stearate                 |
| Manganese phenyl stearate              |
| Aluminum phenyl stearate               |
| Chromium phenyl stearate               |
| Stannous phenyl stearate               |
| Copper phenyl stearate                 |
| Cadmium phenyl stearate                |
| Silver phenyl stearate                 |
| Vanadyl phenyl stearate                |
| Calcium phenyl mercapto stearate       |
| Magnesium phenyl mercapto stearate     |
| Nickel phenyl mercapto stearate        |
| Cobalt phenyl mercapto stearate        |
| Stannous phenyl mercapto stearate      |
| Calcium xenyl stearate                 |
| Magnesium xenyl stearate               |
| Nickel xenyl stearate                  |
| Cobalt xenyl stearate                  |
| Stannous xenyl stearate                |
| Calcium naphthyl stearate              |
| Magnesium naphthyl stearate            |
| Nickel naphthyl stearate               |
| Cobalt naphthyl stearate               |
| Stannous naphthyl stearate             |
| Calcium tolyl stearate                 |
| Magnesium tolyl stearate               |
| Nickel tolyl stearate                  |
| Cobalt tolyl stearate                  |
| Stannous tolyl stearate                |
| Magnesium butyl phthalate (salt-ester) |
| Calcium butyl phthalate (salt-ester)   |
| Nickel butyl phthalate (salt-ester)    |
| Cobalt butyl phthalate (salt-ester)    |
| Aluminum butyl phthalate (salt-ester)  |
| Calcium decyl phthalate (salt-ester)   |
| Cobalt decyl phthalate (salt-ester)    |
| Nickel decyl phthalate (salt-ester)    |
| Stannous decyl phthalate (salt-ester)  |
| Calcium lauryl phthalate (salt-ester)  |
| Cobalt lauryl phthalate (salt-ester)   |
| Nickel lauryl phthalate (salt-ester)   |
| Stannous lauryl phthalate (salt-ester) |
| Magnesium mercapto rosolate            |
| Calcium mercapto rosolate              |
| Nickel mercapto rosolate               |
| Cobalt mercapto rosolate               |
| Aluminum mercapto rosolate             |
| Calcium lauryl rosolate                |

The halogen-bearing salts corresponding to the foregoing halogen-free salts will be found of utility and the following are particularly useful:

|                                  |
|----------------------------------|
| Calcium chlor phenyl stearate    |
| Magnesium chlor phenyl stearate  |
| Calcium chlor naphthyl palmitate |
| Stannous chlor phenyl palmitate  |
| Calcium chlor phenyl laurate     |
| Nickel chlor phenyl laurate      |
| Cobalt chlor phenyl laurate      |
| Stannous chlor phenyl laurate    |
| Calcium chlor phenyl palmitate   |
| Nickel chlor phenyl palmitate    |
| Cobalt chlor phenyl palmitate    |
| Stannous chlor phenyl palmitate  |
| Calcium chlor phenyl myristate   |
| Nickel chlor phenyl myristate    |
| Cobalt chlor phenyl myristate    |
| Stannous chlor phenyl myristate  |
| Calcium chlor naphthyl laurate   |
| Nickel chlor naphthyl laurate    |
| Cobalt chlor naphthyl laurate    |

|                                   |
|-----------------------------------|
| Stannous chlor naphthyl laurate   |
| Calcium chlor naphthyl palmitate  |
| Nickel chlor naphthyl palmitate   |
| Cobalt chlor naphthyl palmitate   |
| Stannous chlor naphthyl palmitate |
| Calcium chlor naphthyl myristate  |
| 5 Sodium chlor naphthyl myristate |
| Nickel chlor naphthyl myristate   |
| Cobalt chlor naphthyl myristate   |
| Stannous chlor naphthyl myristate |
| Calcium chlor xenyl laurate       |
| 10 Sodium chlor xenyl laurate     |
| Nickel chlor xenyl laurate        |
| Cobalt chlor xenyl laurate        |
| Stannous chlor xenyl laurate      |
| Calcium chlor xenyl palmitate     |
| Sodium chlor xenyl palmitate      |
| Nickel chlor xenyl palmitate      |
| Cobalt chlor xenyl palmitate      |
| Stannous chlor xenyl palmitate    |
| Calcium chlor xenyl myristate     |
| 15 Sodium chlor xenyl myristate   |
| Nickel chlor xenyl myristate      |
| Cobalt chlor xenyl myristate      |
| Stannous chlor xenyl myristate    |
| Calcium chlor tolyl laurate       |
| Nickel chlor tolyl laurate        |
| Cobalt chlor tolyl laurate        |
| 20 Stannous chlor tolyl laurate   |
| Calcium chlor tolyl palmitate     |
| Nickel chlor tolyl palmitate      |
| Cobalt chlor tolyl palmitate      |
| Stannous chlor tolyl palmitate    |
| Calcium chlor tolyl myristate     |
| Nickel chlor tolyl myristate      |
| Cobalt chlor tolyl myristate      |
| 25 Stannous chlor tolyl myristate |

Salts of any of the metals of Table XIII with an aromatic acid produced by condensing paraffin wax hydrocarbons with benzoic acid. The salts produced by combining the metals of Table XIII with an aromatic acid such as with benzoic acid, toluic acid or salicylic acid having one or more long aliphatic groups condensed onto the ring structure.

|                           |
|---------------------------|
| 35 Calcium lauryl toluate |
| Nickel lauryl toluate     |
| Stannous lauryl toluate   |

Instead of preparing the salts designed for use as the addition agents of the present invention by treating any of the acids, of the type above identified, with an alkali for example such as sodium hydroxide in the preparation of the corresponding sodium salt of the acid, it is also possible to prepare corresponding salts by first preparing an ester of the acid, and then reacting such ester with an alkali such as sodium hydroxide to prepare, for example, the sodium soap of the acid, and then treating such soap with another salt in the preparation of a salt of a different inorganic radicle. Thus, for example, the methyl ester of chlorphenylstearic acid may be reacted with sodium hydroxide in the production of sodium chlorphenylstearate which is in turn reacted with calcium chloride in the production of calcium chlorphenyl stearate.

It may be preferable to prepare the ester, employed in the foregoing preparation of the salt, where such ester is one of an aromatic acid on page 2 above, by condensing an ester of an aromatic acid with an unsaturated compound or halogenated organic compound instead of condensing the aromatic acid itself with such compound. For example, in the preparation of salts of stearoyl benzoic acid, methyl benzoate may be

60 condensed with stearoyl chloride to form methyl stearoyl benzoate, this ester saponified with sodium hydroxide, and the resulting sodium salt reacted with magnesium chloride in aqueous solution to form magnesium stearoyl benzoate.

65 70 An example of the preparation of magnesium stearoyl benzoate in detail is as follows:

A mixture of 1 mole each of methyl benzoate and stearoyl chloride is dissolved in an equal weight of carbon bisulphide. One mole of anhydrous aluminum chloride is added slowly with

the temperature at 45° C. and the mixture held at that temperature for one hour longer. The materials are then poured into a mixture of cracked ice and concentrated hydrochloric acid, and the carbon bisulphide layer removed and washed with warm water. Carbon bisulphide and moisture are then removed by distilling under vacuum leaving the condensation product, namely methyl stearoyl benzoate. The latter is saponified by adding 1 mole of sodium hydroxide in the form of a 10% aqueous solution, the mixture being refluxed until the aqueous solution is approximately neutral. One-half mole of magnesium chloride is added in the form of an aqueous solution which causes the precipitation of magnesium stearoyl benzoate. The water layer is decanted from the precipitate which is then dissolved in benzol and dried by removing the benzol and water by distilling under vacuum. The resulting product was dissolved in a naphthenic type oil in a concentration of 1% and found to materially improve the oil when used in an internal combustion engine, particularly in preventing the formation of harmful deposits on the piston and piston rings.

Included among the compounds contemplated for use by this invention are stable oil soluble salt-esters of polybasic aromatic acids. These may be formed for example by neutralizing an acid ester of a polybasic aromatic acid with a base, or by partially saponifying a neutral ester of a polybasic aromatic acid with a base so that each molecule of the saponified material retains at least one ester group in addition to at least one basic group.

Examples of such compounds are the salt-esters of the following:

1. Benzene polycarboxylic acids, e. g.  
Phthalic acids  
Trimesic acid  
Trimellitic acid  
Hemimellitic acid  
Pyromellitic acid  
Mellophantic acid  
Prehnitic acid  
Benzene pentacarboxylic acid
2. Naphthalene polycarboxylic acids, e. g.  
Naphthalic acids
3. Pyridine polycarboxylic acids, e. g.  
Lutidinic acid  
Dipicolinic acid  
Cinchomeronic acid  
Isocinchomeronic acid  
Dinicotinic acid  
Alpha-carbocinchomeronic acid  
Beta-carbocinchomeronic acid  
Berberonic acid  
Trimesitinic acid  
Pyridine tetracarboxylic acids  
Pyridine pentacarboxylic acid
4. Pyrrole polycarboxylic acids
5. Quinoline polycarboxylic acids
6. Thiophene polycarboxylic acids
7. Thiazole polycarboxylic acids
8. Diphenyl polycarboxylic acids, e. g.  
Diphenic acid
9. Dibenzyl polycarboxylic acids
10. Anthracene polycarboxylic acids
11. Phenanthrene polycarboxylic acids
12. Thianthrene polycarboxylic acids

Where such salt-esters are employed, it will generally be found advantageous to have at least one of the ester groups consist of an aliphatic or cyclo-aliphatic group and preferably one containing four or more carbon atoms. For example, salts of the acid butyl or amyl esters of phthalic acid have been found suitable.

Specific examples of these salt-esters have been so labeled in the principal list of specific examples given above.

In view of the particular uses for which my compounded lubricants are intended, it is apparent that of the salts included in the foregoing enumeration of the addition agents which may be employed, those which are readily oil-

soluble are the ones preferred for use. When these compounded oils are designed for use under conditions where high temperatures are usually encountered, the addition agents should be stable at elevated temperatures. For use in crankcase lubricants for internal combustion engines, they should preferably be stable to the extent where there will be substantially no decomposition, when the lubricating composition 10 is exposed to temperatures up to 250° F.

The addition agents which are to be selected from the class described should be such that they are relatively non-corrosive with respect to the metallic surfaces with which they come in 15 contact during use. Certain of the named addition agents may be found to be detrimentally corrosive to certain sensitive bearing metals, in which case an appropriate corrosion inhibitor may be employed in conjunction therewith in 20 the composition.

A lubricating composition prepared in accordance with my invention and which is predominantly hydrocarbon oil may contain from an effective amount to 20% of the salt addition agent 25 above identified. In general, it will be found that an amount as low as .1% will often be quite effective and that amounts in excess of 10% are seldom necessary. A preferred range of concentrations for the salt in the oil is from .25% to 30 about 2%.

The principal use for which the lubricants of this invention are designed is in the crankcase of internal combustion engines. The oil base is therefore preferably a liquid highly refined mineral oil with the addition agent present therein in such amounts as not to detrimentally change the viscosity of the composition. The viscosity of the blended lubricant used for this purpose may vary from an S. A. E. 10 grade to an S. A. E. 50. Generally the blended lubricant in the viscosity range of S. A. E. 10, 20 and 30 will be found of most general utility.

It is also within the contemplation of this invention to provide the addition agents in the 45 form of a concentrate in a suitable oil, said oil containing rather high percentages of the addition agents. Such concentrates may be employed for further blending with a lubricating oil in the proportions desired for the particular 50 conditions of use.

While mineral oil, generally, is the principal ingredient of the lubricant, it is not essential that it be the only ingredient other than the addition agents, provided that there be no additional ingredient which is incompatible with such addition agent. It is within the contemplation of this invention to include, if necessary or desirable, such other addition agents as are commonly added to improve the viscosity index 60 or cold test of the lubricants; addition agents which function as corrosion inhibitors; as well as addition agents whose property is to reduce the tendency of the composition toward oxidation; and a lubricating composition according 65 to this invention which also has a separate film-strength or oiliness increasing agent has been found to be especially effective.

When used in conjunction with a hydrocarbon lubricating oil, it is obvious that, generally, 70 only such amounts of the addition agent may be included as are soluble in the specified amount of oil. By the term "soluble," as herein used, it is intended to indicate the ability to form not only true solutions but also any form 75 of substantially permanently homogeneous

composition when incorporated in mineral oil. With most of the compounds there is usually little difficulty, especially if the incorporation is effected in the manner described in Cornell Patent No. 2,042,880, and since quite small percentages often give remarkably improved results, it is seldom of extreme importance that the addition agents be oil-soluble in all proportions.

The addition agents above enumerated for use in my compounded lubricants include certain ones which may be found to at least partially decompose under conditions of extreme stress such as the very high temperature encountered in certain classes of use, while others are quite stable even under such extreme conditions.

The use for which the lubricant is designed therefore determines the particular type of addition agent to be selected. A certain amount of decomposition, which proceeds at a relatively slow rate, is usually not harmful. Care should be exercised, however, to select for a particular set of operating conditions, an addition agent which in the oil base used, will not decompose under such operating conditions except at a low rate.

By the term "stable" as used herein in describing the addition agents is meant the characteristic of the addition agents which enables them to resist decomposition in the oil under the condition of use for which the lubricating composition is designed.

The lubricating compositions of this invention may be prepared by first preparing the salt and then dissolving the salt in the oil base, or they may be prepared by reacting the acid in solution in all or a portion of the oil with a suitable basic compound in order to form the desired salt directly in solution in oil. In the latter case, it is frequently desirable to remove the water formed by the reaction, or which may have been added with the basic compound, by some means such as by heating at atmospheric or sub-atmospheric pressure.

In case the salt to be used is water-insoluble, an alternative procedure is as follows:

An aqueous solution of a water-soluble salt of the acid is first prepared, for example by dissolving the acid in an aqueous solution of caustic soda or caustic potash. The aqueous salt solution is then emulsified with oil and a water soluble salt containing the cation of the desired salt is added to the mixture. The desired salt is thus precipitated from the aqueous medium and subsequently or simultaneously dissolved by the oil medium. Separation of the aqueous and oil layers is then effected for example by settling or centrifuging. Subsequent water-washing of the oil solution to remove traces of inorganic salts may be desirable, and removal of moisture may also be required.

A preferred class of addition agents for use in improved lubricating compositions of my invention may be defined as salts of aromatic acids, which salts contain the radicle  $-C-X-M$  in which X is an element of the class consisting of oxygen and sulphur and M is a member of the class consisting of metals and basic radicles.

This application is a continuation-in-part of my aforesaid co-pending applications Serial Numbers 737,070, 245,226 now Patent No. 2,223,127, 332,782 now Patent No. 2,223,129, 332,781 now Patent No. 2,223,128, 334,082 now Patent No. 2,223,130, and 216,153, the latter being in turn

a continuation-in-part of Serial No. 760,038 now Patent No. 2,121,825.

Other modes of applying the principle of the invention may be employed, change being made as regards the details described, provided the features stated in any of the following claims or the equivalent of such be employed.

I, therefore, particularly point out and distinctly claim as my invention:

- 10 1. A liquid lubricating composition comprising a major proportion of mineral lubricating oil and an oil-soluble salt of an aromatic acid in an effective amount insufficient, however, to substantially change the viscosity of the composition.
- 15 2. A liquid lubricating composition comprising a major proportion of mineral lubricating oil and an oil-soluble salt of an aromatic acid in an amount from .10% to less than that which would substantially change the viscosity of the composition.
- 20 3. A liquid lubricating composition suitable for use as the lubricant for the crankcase of internal combustion engines comprising a major proportion of highly refined mineral lubricating oil to which has been added an effective minor amount of an oil-soluble salt of an aromatic acid without any substantial change in the viscosity of the refined mineral lubricating oil.
- 25 30 4. The method of reducing the rate of deposit in internal combustion engines of those materials usually resulting from the use of highly refined mineral lubricating oil as the primary lubricant which consists in incorporating in such lubricant a minor amount of an oil-soluble salt of an aromatic acid.
- 35 40 5. The method of reducing the rate of deposit on the pistons in internal combustion engines of those materials usually resulting from the use under high temperatures of highly refined mineral lubricating oils as the primary lubricants, which consists in introducing to the area where such deposits tend to occur, a minor amount of an oil-soluble salt of an aromatic acid.
- 45 50 6. A liquid lubricating composition comprising a major proportion of mineral lubricating oil and a minor amount of an oil-soluble polyvalent metallic salt of an aromatic acid.
- 55 7. A lubricating composition comprising a major proportion of mineral lubricating oil and a minor proportion of an oil-soluble salt of an aromatic acid of the class having a carboxyl group attached to the ring.
- 60 8. A lubricating composition comprising a major proportion of mineral lubricating oil and a minor proportion of an oil-soluble salt of a substituted benzoic acid.
- 65 9. A lubricating composition comprising a major proportion of mineral lubricating oil and a minor proportion of an oil-soluble salt of a substituted salicylic acid.
- 70 10. A lubricating composition comprising a major proportion of mineral lubricating oil and a minor proportion of an oil-soluble salt of an aromatic substituted carboxylic acid.
- 75 11. A lubricating composition comprising a major proportion of mineral lubricating oil and a minor proportion of an oil-soluble salt of an aromatic acid of the class consisting of sulphur-containing aromatic-substituted aliphatic acids.
- 80 12. A lubricating composition comprising a major proportion of mineral lubricating oil and a minor proportion of an oil-soluble salt of an aromatic acid of the class consisting of hydroxyl containing derivatives of triphenyl methane.

13. A lubricating composition comprising a major proportion of mineral lubricating oil and a minor proportion of an oil-soluble salt of an aromatic acid having a molecular composition like that produced by condensing an aromatic heterocyclic compound with an aliphatic acid.

14. A lubricating composition comprising a major proportion of mineral lubricating oil and a minor proportion of an oil-soluble salt of an aromatic acid having a molecular composition like that produced by condensing an oxygen bearing aromatic compound with an aliphatic acid.

15. A lubricating composition comprising a major proportion of mineral lubricating oil and a minor proportion of an oil-soluble salt of an aromatic acid having a molecular composition like that produced by condensing an aromatic acid with an unsaturated aliphatic oxygen compound.

16. A lubricating composition comprising a major proportion of mineral lubricating oil and a minor proportion of an oil-soluble salt of an aromatic acid having a molecular composition like that produced by condensing an aromatic acid with an unsaturated halogen bearing aliphatic compound.

17. A lubricating composition comprising a major proportion of mineral lubricating oil and a

minor proportion of an oil-soluble salt of an aliphatic substituted aromatic acid in which the aliphatic substituent contains oxygen.

18. A lubricating composition comprising a major proportion of mineral lubricating oil, and a minor proportion of an oil-soluble salt of an aromatic acid having a molecular structure like that produced by condensing a salicyclic acid with oleyl alcohol.

19. A lubricating composition comprising a major proportion of mineral lubricating oil, and a minor proportion of an oil-soluble polyvalent metallic salt of an aromatic acid having a molecular structure like that produced by condensing salicylic acid with oleyl alcohol.

20. A lubricating composition comprising a major proportion of mineral lubricating oil, and a minor proportion of an oil-soluble salt of an aromatic acid having a molecular structure like that produced by condensing an oxygen bearing aromatic derivative of furan with an aliphatic acid.

21. A liquid lubricating composition comprising a major proportion of mineral lubricating oil, and a minor amount of an oil-soluble metallic salt of an aromatic acid.

CARL F. PRUTTON.